

Jan. 11, 1927.

1,613,726

H. W. SANFORD

ART OF ANNEALING METAL

Filed Feb. 11, 1922

5 Sheets-Sheet 1

FIG. 1.



FIG. 2.



FIG. 3.



Inventor

Hugh W. Sanford  
By Cyrus K. Lehr  
Attorney

Jan. 11, 1927.

**1,613,726**

**H. W. SANFORD**

## ART OF ANNEALING METAL

Filed Feb. 11, 1922

5 Sheets-Sheet 2

FIG. 4.



Hugh W. Sanford

*Cyrus Kehr* attorney

Jan. 11, 1927.

1,613,726

H. W. SANFORD

ART OF ANNEALING METAL

Filed Feb. 11, 1922

5 Sheets-Sheet 3

Fig. 5.



Hugh W. Sanford

By

James Reiter

Attorney

Jan. 11, 1927.

1,613,726

H. W. SANFORD

ART OF ANNEALING METAL

Filed Feb. 11, 1922

5 Sheets-Sheet 4

FIG. 6.



Hugh W. Sanford  
Oscar R. Elie, attorney

Jan. 11, 1927.

1,613,726

H. W. SANFORD

ART OF ANNEALING METAL

Filed Feb. 11, 1922

5 Sheets-Sheet 5

FIG. 7.



FIG. 8.



FIG. 9.



Inventor

Hugh W. Sanford  
By *Oscar Kellar* Attorney

Patented Jan. 11, 1927.

1,613,726

# UNITED STATES PATENT OFFICE.

HUGH W. SANFORD, OF KNOXVILLE, TENNESSEE.

## ART OF ANNEALING METAL.

Application filed February 11, 1922. Serial No. 535,835.

My improvement relates especially to apparatus and methods for annealing metal castings and forgings.

The object of my improvement is to provide means and a method for carrying on such an annealing operation under control, in order that the castings may be brought to the desired high temperature and then cooled in such manner and under such control as will cause the cooling to be uniform.

According to the method heretofore practiced and now in general use, the hot castings are put into a closed chamber until such time as it is assumed that the castings have been sufficiently "soaked" and sufficiently cooled to effect the intended treatment, the chamber being filled with stagnant gases—gases which do not move in the chamber excepting as movement is caused by difference in temperature. In other words, such gases do not positively circulate or travel through the chamber. This method is not satisfactory (1) first, because the castings are required to be in the pit a long time, usually about six days; (2) second, because it is well known that the cooling of the castings is irregular and uneven, and internal strains, due to uneven shrinkage, are found to exist in the castings.

Generically speaking, my improved method involves the surrounding of the castings with a fluid medium and relatively moving the fluid medium and the castings, whereby the fluid medium is adapted to deliver heat to or take heat from the castings by contact with the castings. That is to say, if at the beginning of the operation the temperature of the castings is not sufficiently high to effect the annealing, the relative stream of the fluid medium may be hotter than the castings, whereby the castings will receive heat from the fluid medium and gradually attain the desired high temperature. And when the castings are at the desired high temperature, either at the time they are put into the pit or subsequently made so by contact with the high temperature fluid medium, the temperature of the relative stream of the fluid medium is gradually reduced until the castings have been sufficiently cooled for removal. This period is to be made of such duration as will allow the annealing change and also allow the substantially uniform elimination of heat from all parts of the castings, in order that internal shrinkage strains may be substantially avoided.

The fluid medium may be ordinary atmospheric air, or it may be the waste air and other gases from a cupola or other metallurgical furnace, or it may be a gas or combination of gases other than those mentioned. For example, if, in the treatment of some castings, it is desirable to avoid the oxygen of the atmosphere, then nitrogen or carbon dioxide, or some other gas having no free oxygen may be used. In some cases it may be desirable to artificially prepare the fluid medium. For example, if atmospheric air is used, it may be desirable to mingle therewith some other gas or gases or vapor or vapors adapted to exert some physical or chemical effect upon the castings or adapted to prevent some other constituent from exerting an undesirable physical or chemical effect upon the castings. And, at low heat, the fluid medium may be water or oil or other liquid. If the fluid medium is a liquid, it may be desirable to introduce into the liquid a constituent or constituents intended to act favorably upon the castings or to prevent another constituent or constituents from acting unfavorably upon the castings.

In every form of the operation, there is relative movement between the fluid medium and the castings, and such movement is positive and directed and controlled in such manner as to compel the change of temperature—either increasing or diminishing—to be substantially uniform relative to all parts of the castings and relative to the rate of such change.

In the accompanying drawings,

Fig. 1 is a diagrammatic plan illustrating an apparatus adapted to be used for treating metal castings by my improved method;

Fig. 2 is a diagrammatic plan of a similar apparatus;

Fig. 3 is a diagrammatic plan of another similar apparatus;

Figs. 4, 5 and 6 are diagrammatic plans illustrating apparatus containing a plurality of annealing chambers;

Figs. 7, 8 and 9 illustrate modifications, Fig. 9 being a vertical section on the line, 9—9, of Fig. 7.

Referring first to Fig. 1 of said drawings, A is a pit or chamber into which castings are to be placed for annealing. G is a pipe or duct leading from said chamber and opening into the atmosphere. G<sup>1</sup> is a valve or gate for controlling the movement of the fluid medium from the chamber, A, through the

duct, G. D is a cupola or other furnace from which waste heated air or other gases may be taken. C is a pipe or duct leading from the cupola or furnace to the fan, F. B is a pipe or duct leading from the fan into the annealing chamber, A, opposite the discharge pipe or duct, G. On the pipe or duct, C, is a branch duct, E, communicating with the atmosphere. In said branch duct is a valve or gate, E<sup>1</sup>, by means of which admission of air into said branch may be controlled.

10 The chamber and the ducts should be so constructed as to reduce seeping or leakage and thermal conduction, in order that the 15 temperatures of the fluid medium in the chamber or ducts may be maintained with the least interference from temperature of the outside atmosphere.

10 The operation of this apparatus is as follows:

20 The castings to be annealed are placed into the annealing chamber, A, at any convenient temperature. Then said chamber is closed from the atmosphere. Then the gate, 25 G<sup>1</sup>, is opened and the fan, F, is set into motion for drawing hot gases from the cupola or furnace, D, through the duct, C, and driving said gases through the duct, B, into and through the annealing chamber and the 30 duct, G.

35 The adjustment of rapidity of such movement should depend upon the temperature of the castings in the annealing chamber and upon the temperature of the fluid medium 40 passing from the duct, B, into the annealing chamber. If the castings need be brought to a higher temperature than they have when put into the chamber, and the gases issuing from the furnace or cupola are at a sufficiently 45 high temperature for the purpose, the fan, F, and the gate, G<sup>1</sup>, are controlled to allow the absorption of heat by the castings from the fluid medium. If the temperature of the castings is already sufficiently 50 high, air is to be admitted through the branch duct, E, to mingle with the gases from the cupola, whereby the temperature of the fluid medium is reduced, to adapt it to take heat from the castings. Hence the 55 gates, G<sup>1</sup> and E, and the fan are so controlled as to deliver the fluid medium through the annealing chamber at approximately the temperature of the castings, and thereafter the adjustment of said gates and the 60 velocity of the fan are varied to reduce the temperature of the fluid medium in the annealing chamber gradually and at such rate as will cause uniform passing of heat from the castings into the fluid medium and as will subject the castings to the action of heat during a period of such duration as will be sufficient to anneal the castings.

65 It is to be observed that the required temperature of the fluid medium in the duct, C, will depend upon the effectiveness of the

70 thermal insulation of said duct and the duct, B, and the chamber, A. That is to say, if there is gas leakage or temperature conduction through the walls, the temperature of the fluid medium going through the duct, C, must be sufficiently high to compensate for heat loss through leakage or conduction.

75 At this point it is also to be observed that the gate, G<sup>1</sup>, and the fan, F, may be made to co-operate to prevent the inward seeping or leakage of colder atmospheric air through the walls of the duct, B, and through the walls of the annealing chamber, A. For this purpose, the gate, G<sup>1</sup>, is to be open far enough to permit the passage of the fluid 80 medium when the latter is under such pressure in the annealing chamber and the duct, B, as will balance or exceed the inward pressure of air from the outer atmosphere. If such outward pressure exceeds the inward pressure, there will be outward seeping or leakage, and the entrance of colder air will be prevented. By the method heretofore in use, the leakage of atmospheric air into the pit is not avoided. On the contrary, cold 85 air may seep into the pit and drive out warm air. Furthermore, the gradual cooling of the contents of the pit causes the condensation of the air in the pit, whereby a partial 90 vacuum is created and inward movement of air from the atmosphere is induced.

95 In Fig. 2, the apparatus is the same as in Fig. 1, excepting that a gate, C<sup>1</sup>, is put into the duct, C, adjacent the cupola and a duct, H, is placed with one end opening into the 100 duct, G, while its other end opens into the duct, C. In each end of this duct, H, is a gate, H<sup>1</sup>.

105 This form of the apparatus contemplates at times omitting the use of hot gases coming from the cupola. For example, if the castings in the annealing chamber are already at a high temperature, and said chamber and the ducts are well insulated, it is to be expected that the gases issuing from the 110 annealing chamber into the duct, G, will be so highly heated that they may be made to circulate thence through the ducts, H, C and B, and again into the annealing chamber with only the reduction of temperature suitable 115 for the reduction of temperature in the castings. In such a case, the fluid medium may be circulated continuously, heat being gradually taken from the castings in the annealing chamber until the elapse of the desired annealing period and the desired reduction of temperature in the castings. For such operation the gates, G<sup>1</sup> and E<sup>1</sup>, are closed and the gates, H<sup>1</sup>, are opened. If the 120 cooling in the annealing chamber is to be hastened, the gates, G<sup>1</sup> and E<sup>1</sup>, may be partially opened, the partial opening of the gate, G<sup>1</sup>, being for the purpose of allowing the escape through the duct, G, of gases to 125 compensate for the air taken in through the 130

duct, E. But it is to be preferred that the flow through the duct, G, be retarded sufficiently to cause the gas pressure in the annealing chamber to equal or exceed outside atmospheric pressure, in order that, as above stated, inward leakage of air will be avoided.

But if it is deemed that the temperature in the annealing chamber is being reduced too rapidly while the gates, E<sup>1</sup> and G<sup>1</sup>, are yet closed, the gate, C<sup>1</sup>, may be partly open, so that some heated gases will be drawn from the cupola to mingle with the gases coming through the duct, H.

In the form shown by Fig. 3, the fluid medium receives heat only in a stove, D, and from the hot castings in the annealing chamber, the stove being of "checker-work" or other form heretofore used for heating air before its admission into a metallurgical cupola or blast furnace. Or the stove may contain any form of electric heating means.

In this form, the annealing chamber, A, and the duct, H, and the fan, F, are present as in Fig. 2; but the duct, H, communicates directly with the fan. From the fan a duct, I, leads into the stove, D, and from the stove, a duct, B, leads into the annealing chamber, A. A by-pass duct, J, leads from the duct, I, to the duct, B. Between the by-pass duct and the stove, the duct, I, has a gate or valve, I<sup>1</sup>; and the by-pass duct, J, has a gate or valve, J<sup>1</sup>. The duct, B, has a gate, B<sup>1</sup>, between the stove and the by-pass duct, J. The duct, H, has a gate, H<sup>1</sup>, near the annealing chamber. On the duct, H, is a branch duct, K, which opens into the atmosphere. In said branch is a gate or valve, K<sup>1</sup>. And on the duct, H, near the annealing chamber, is a branch duct, K<sup>2</sup>, in which is a gate, K<sup>2</sup>.

The operation of this form of apparatus is as follows:

The castings are placed into the annealing chamber. Then the chamber is closed. Then the fan is set into action, whereby the air is driven through the duct, I, and the stove and the duct, B, into the annealing chamber, the gates, I<sup>1</sup> and B<sup>1</sup>, being open and the gate J<sup>1</sup>, being closed; or the air is driven from the duct, I, through the by-pass duct, J, into the duct, B, and thence into the annealing chamber, the adjustment of said gates being reversed; or, if less heat is desired, a part of the air may be driven through the stove and a part through the by-pass duct, the gates, B<sup>1</sup>, I<sup>1</sup> and J<sup>1</sup>, being partially opened.

The gate, H<sup>1</sup>, in the duct, H, may be closed to any extent desired for the purpose of retarding flow of fluid medium out of the annealing chamber, in order that there may be outward fluid medium pressure in the annealing chamber for avoiding inward seeping or leaking of cool or cold atmospheric air. The function of the branch duct, K,

on the duct, H, is to admit atmospheric air into the circulation when it is desirable to hasten the reduction of the temperature of the fluid medium. In such case, the gate, K<sup>1</sup>, is to be opened sufficiently to admit the desired stream of atmospheric air, the gate, K<sup>2</sup>, on the branch duct, K<sup>2</sup>, is opened far enough to permit escape of enough fluid medium to compensate for air taken in through the branch, K. When no air is to be thus added to the circulation, the gate, K<sup>1</sup>, is to remain closed.

In Fig. 4, a group of annealing chambers, A<sup>1</sup>, A<sup>2</sup>, A<sup>3</sup>, A<sup>4</sup> and A<sup>5</sup>, similar to the annealing chamber, A, are arranged to receive fluid medium circulation from a common circulation stream. These chambers are arranged parallel to each other in a straight row, their ends leading to common lines.

From the fan, F, a duct, L, extends parallel to the left hand ends of the five chambers. Branch ducts L<sup>1</sup>, connect the duct, L, with the respective chambers. From a stove, D, a duct, O, leads to the fan. From the stove a duct, M, extends parallel to the right hand ends of the annealing chambers. Branch ducts, M<sup>1</sup>, connect the duct, M, and the respective annealing chambers. Between the stove, D, and the chamber, A<sup>1</sup>, a by-pass duct, N, extends from the duct, M, to the duct, O. In the branch ducts, L<sup>1</sup>, connecting the main duct, L, and the annealing chambers are gates, L<sup>2</sup>. Between the branch ducts, L<sup>1</sup>, gates, L<sup>3</sup>, are placed in the main duct, L. In the branch ducts, M<sup>1</sup>, are placed gates, M<sup>2</sup>. In the main duct, M, between the branch ducts, M<sup>1</sup>, are placed gates, M<sup>3</sup>. Between the stove, D, and the by-pass a gate, M<sup>3</sup>, is also placed in the main duct, M. In the by-pass duct, N, is a gate, N<sup>1</sup>. In the duct, O, is a gate, O<sup>1</sup>. On the duct, O, is a branch, P, communicating with the atmosphere. In said branch is a gate, P<sup>1</sup>.

In operation, if the fluid medium is to pass through all the annealing chambers, the gates, L<sup>3</sup>, and the gates, L<sup>2</sup>, are to be opened so as to allow the fluid medium to be driven from the fan through the entire length of the main duct, L, in the branch ducts, L<sup>1</sup>, and the branch ducts, M<sup>1</sup>, are to be opened to such extent as will give to each annealing chamber the desired flow of fluid medium. For example, if the chamber, A<sup>5</sup>, is filled with castings having the maximum temperature, the adjacent gate, M<sup>2</sup>, may be nearly closed and the adjacent gate, L<sup>2</sup>, opened only far enough to admit enough fluid medium to cause sufficient pressure within that chamber to resist and avoid inward seeping or leaking of external air. This may be continued until it is desired to begin the cooling of the castings in that chamber. Then the gates, M<sup>2</sup> and L<sup>2</sup>, are to be adjusted to establish the desired flow of fluid medium through that

chamber. And if the castings in another chamber are so nearly cooled as to make desirable a larger flow of fluid medium through that chamber, the gates at that 5 chamber are to be adjusted to allow the largest flow through that chamber. When a chamber is to be emptied or charged, the gates at that chamber are to be entirely closed.

10 The fluid medium issuing from the annealing chambers through the branch ducts, M<sup>1</sup>, into the main duct, M, follow that duct toward the stove, D, and pass through that stove, and the duct, O, to the fan, if the 15 gate, N<sup>1</sup>, in the by-pass, N, is closed, and the gate, M<sup>3</sup>, adjacent the stove is open. If the position of those gates is reversed, the flow will be through the by-pass duct and not through the stove. In that case, 20 the gate, O<sup>1</sup>, in the duct, O, should also be closed, in order to avoid the eduction of air or other gases from the stove. If it is desired to heat or re-heat only a portion of the fluid medium coming along the 25 main duct, M, the gates, M<sup>3</sup>, N<sup>1</sup> and O<sup>1</sup>, may be partially opened in such relation to each other as to cause a part of the fluid medium to pass through the stove while the other part moves through the by-pass duct. 30 From the foregoing it will be seen that this multiple annealing chamber apparatus is adapted to large and economical capacity; and that any one of the several chambers may be given the desired flow of the fluid 35 medium and that any of the chambers may at any time be completely cut off from the circulation of the fluid medium. And it will be observed that by the alternating charging and discharging of the annealing 40 chambers there should always be one or more highly heated chambers adapted to heat the circulating fluid medium, so that ordinarily it will not be necessary to pass the fluid medium through the stove, D. And 45 it will be observed that provision is made by means of the branch, P, for reducing the temperature of the circulating fluid medium, if that medium receives excessive heat by passing through the hot annealing 50 chambers.

In Figs. 5 and 6, the structure is the same as in Fig. 4 with the addition of an outer main duct, Q, extending parallel to the main duct, L, and an outer main duct, S, extending parallel to the main duct, M. Each end of the main duct, Q, connects with the duct, L, and each end of the main duct, L, connects with the main duct, M. At each junction of the duct, Q, is a gate, Q<sup>1</sup>, and at each junction of the duct, S, with the duct, M, is a gate, S<sup>1</sup>.

When the gates, Q<sup>1</sup> and S<sup>1</sup>, are closed, this apparatus may be operated in the manner described concerning the apparatus of 65 Fig. 4. But by an appropriate setting of

the gates, the fluid medium may be moved serially through the annealing chambers, beginning with the chamber, A<sup>1</sup>. For this the gates, Q<sup>1</sup>, are to be closed and the gates, S<sup>1</sup>, opened, and all the gates L<sup>2</sup> and M<sup>2</sup> 70 opened, and the alternate gates, L<sup>3</sup>, opened, beginning with the gate, L<sup>3</sup>, between the fan and the adjacent branch duct, L<sup>1</sup>, and closing the alternate gates, M<sup>3</sup>, beginning with the gate between the by-pass duct, N, 75 and the adjacent branch duct, M<sup>1</sup>. When the gates have been so arranged, the fluid medium may take the course indicated by the arrows in Fig. 5; namely from the fan through the chamber, A<sup>1</sup>, into the main duct, 80 M, and thence through the chamber, A<sup>2</sup>, and thence into the main duct, L, and along said duct into and through the chamber, A<sup>3</sup>, and again into the main duct, M, and along 85 said duct and into and through the chamber, A<sup>4</sup>, and then into the main duct, L, and through the chamber, A<sup>5</sup>, and the branch duct, M<sup>1</sup>, into the outer main duct, S, and through the length of that duct into the 90 duct, M, adjacent the stove, and thence 90 through the stove or through the by-pass duct, N, or through both of these members (according to the setting of the gate, N<sup>1</sup>, and the adjacent gate, M<sup>3</sup>), into the 95 duct, O, and again into the fan. 95

In Fig. 6, the gates are set to reverse the circulation above described. The fluid medium then passes from the fan through the adjacent part of the main duct, L, and thence into and through the length of the outer main duct, Q, and through the adjacent branch duct, L<sup>1</sup>, and then through the chamber, A<sup>5</sup>, the main duct, M, the chamber, A<sup>4</sup>, the main duct, L, the chamber, A<sup>3</sup>, the main duct, M, the chamber, A<sup>2</sup>, the main duct, L, and the chamber, A<sup>1</sup>, into the main duct, M, and through the stove or the by-pass duct, or through both said members (according to the setting of the gate, N<sup>1</sup>, and the adjacent gate, M<sup>3</sup>), into the 100 duct, O, and again into the fan. 110

By thus reversing the circulation, the flow can be adapted to the heat in the chambers.

The circulation may be further varied by closing the gates leading into any two of 115 five chambers; for example, by closing the gates leading into the chambers, A<sup>4</sup> and A<sup>2</sup>. When that has been done, the flow will be through the remaining chambers. For such variation it is only necessary that an odd 120 number of chambers be left open.

This variation in circulation permits the 125 charging and discharging of any chamber without suspending circulation through other chambers.

In Fig. 7 provision is made for passing the fluid medium into the annealing chamber, A, at different points. The duct, T, has branches, T<sup>1</sup>, one of which extends along each side wall of the chamber, Ports. T<sup>2</sup>, 130

in the chamber walls afford communication between the branch ducts and the interior of the chamber. In said ports are gates,  $T^3$ . These gates are to be opened to admit the fluid medium to different parts of the interior of the chamber, as may be found desirable for successful operation. Not only may the fluid medium be thus admitted into the chamber at different places, but the 10 quantities admitted at the different ports may be varied by partially closing the gates.

In Fig. 8, a duct,  $U$ , leads into one end wall of the annealing chamber, and a duct,  $U^1$ , leads outward from the opposite end wall of 15 said chamber. Near the admission end wall of the chamber is an upright cross wall,  $U^2$ , in which are ports,  $U^3$ , in which are gates,  $U^4$ . Near the opposite end wall is a similar upright cross wall,  $U^6$ , in which are 20 ports,  $U^6$ , in which are gates,  $U^7$ . When all these gates are opened, the fluid medium entering through the duct,  $U$ , will pass through all the ports,  $U^3$ , and through the chamber,  $A$ , and then through all the ports,  $U^6$ , and out through the duct,  $U^1$ . But any 25 of the gates may be closed or partially closed to vary the flow of fluid medium as may be found desirable to reach all the castings in the chamber.

30 Furthermore, deflecting plates,  $T^4$ , may be placed on the inner face of the walls of the annealing chamber, as shown in Figs. 7, 8 and 9, in such positions and at such inclinations as will cause the desired movement of the fluid medium to all parts of the mass of castings in the chamber.

It is also to be observed that, in addition to the mechanical means described for effecting a distribution of the fluid medium 40 in the annealing chamber, delivering the fluid medium into the annealing chamber under pressure will aid in driving the fluid medium to all parts of the interior of said chamber, and hence to all parts of the stack 45 of castings in the chamber. For such an operation it is specially desirable that there be in the chamber no space in which the fluid medium is stagnant. Thus delivering the fluid medium into the chamber serves 50 the double purpose of (1) moving said medium through all parts of the chamber and (2) preventing inward leakage of atmospheric air into the chamber.

Regarding the last above-mentioned feature, it is to be noted that complete control 55 of the operation can be had only by provision for preventing such inward leakage. For the outside atmosphere varies in temperature at different times, and if there is leakage into the annealing chamber, the quantity of air thus entering the chamber may be unequal in different parts of the chamber. By substantially avoiding such inward leakage and taking atmospheric air 60 into the ducts, when cooling is desired, all

parts of the interior of the annealing chamber will receive the fluid medium at the same temperature, and that temperature is under the control of the operator. He can observe the temperature of the fluid medium in the 70 duct which discharges into the chamber. If he finds that temperature too high, he can admit atmospheric air into the duct. If he finds the temperature too low, he can attend to the heating of the fluid medium before it is discharged into the chamber. 75

Regarding the heating of the fluid medium outside of the annealing chamber, it is to be observed that the cupola or furnace and the stove above described perform the 80 same function and are heaters or heating means external to the annealing chamber. It has already been indicated that the means for producing heat in the heaters may be varied. If the heater is a metallurgical 85 cupola or furnace, then the heat is derived from the operation carried on in the cupola or furnace. If the heater is such a "stove" as has been described, the interior of that stove is ordinarily heated by means of gas, 90 or devices for developing heat by electricity may be used, preferably by placing them into the stove.

It is to be understood that pieces of metal other than castings may be placed into the 95 annealing chambers for the treatment herein described, the operation then being varied as may be required for the particular kind of metal. Hence what has been said herein regarding castings is applicable also to other 100 metals which are to be annealed.

Those who are familiar with this art will understand that the annealing of thick pieces of metal will require longer time than is required for smaller pieces, and that the 105 operation will have to be regulated accordingly.

It is thought well to also specifically direct 110 attention to the fact that variation in the operation may be effected by merely varying the velocity of the stream of fluid medium. If the flow is rapid, the contact between the fluid medium and any metal surface in the chamber will be of short duration and hence only a relatively small quantity of heat can be imparted to that part of the fluid medium from that surface. But immediately thereafter another portion of the fluid medium, ready to receive heat, is taking 115 heat from the same surface. Thus there is a rapid elimination of heat from that surface with only a limited addition of heat to every part of the stream of fluid medium. If, in such a case, the rate of elimination of heat from the metal is to be reduced, that 120 can be accomplished by reducing the velocity of the stream of fluid medium.

It will now be seen that for the treatment 125 of the metal, reliance is placed upon the circulating or traveling fluid medium which, 130

in the form of a stream, surrounds the metal and receives heat from or imparts heat to the metal, depending upon whether the temperature of the fluid medium is lower or higher than the temperature of the metal, the fluid medium being heated by means extraneous to the metal, if the temperature of the fluid medium is not as high as desired, or the fluid medium being at times, by means 10 extraneous to the metal, kept at a uniform temperature, when it is desired to keep the metal at a uniform temperature during a prolonged interval, and the heat received by the fluid medium from highly heated 15 metal being at times utilized in the treatment of other metal surrounded by said stream after said stream has left the highly heated metal.

I claim as my invention,

20 1. The herein-described method of annealing metal, which method consists in excluding the metal from the atmosphere, then relatively moving the metal and a fluid medium of higher temperature than the temperature of the metal, whereby the metal is surrounded by said fluid medium of high temperature and the metal is raised to a temperature high enough for annealing, and then gradually reducing the temperature 25 of the fluid medium for the gradual elimination of heat from the metal, substantially as described.

2. The herein-described method of annealing metal, which method consists in excluding the metal from the atmosphere, then relatively moving the metal and a fluid medium of higher temperature than the temperature of the metal, whereby the metal is surrounded by said fluid medium of high 30 temperature and the temperature of the metal is raised high enough for annealing, and then gradually accelerating the elimination 35 of heat from the metal by increasing the velocity of the relative movement of the metal and the fluid medium, substantially as described.

3. The herein-described method of annealing metal, which method consists in excluding said metal, when at annealing heat, 40 from the atmosphere and establishing an endless stream of fluid medium, a portion of which stream surrounds said metal, the temperature of the fluid medium of said

endless stream being lower than the temperature of said metal, a part of the fluid 55 medium of said endless stream being discharged into the atmosphere and other fluid medium being added to said stream, substantially as described.

4. The herein-described method of annealing metal, which method consists in isolating a plurality of masses of metal when at annealing heat from the atmosphere and from each other, and then moving a stream of fluid medium to and around one of said masses and then moving the same stream to and around another of said masses for the controlled reduction of temperature of the metal, substantially as described.

5. The herein-described method of annealing metal, which method consists in forming a plurality of groups of metal, when at annealing heat, the metal of one group being of a higher temperature than the metal of another group and the latter requiring higher temperature, then passing a fluid medium stream to and around the metal group of higher temperature and then moving the same fluid medium to and around another group, whereby said fluid medium will acquire a higher temperature while surrounding the first group and thereby be adapted to impart heat to the second group and then slowly cooling said metals, substantially as described.

6. The herein-described method of annealing metal, which method consists in contacting metal, when at annealing heat, with a cooler fluid medium and then contacting said fluid medium with metal of lower temperature whereby the latter metal is heated, and then slowly cooling said metals, substantially as described.

7. The herein-described method of annealing metal, which method consists in contacting metal, when at annealing heat, with an endless stream of cooler fluid medium and then contacting said fluid medium with metal of lower temperature whereby the latter metal is heated, and then slowly cooling said metals, substantially as described.

In testimony whereof I have signed my name, this first day of February, in the year one thousand nine hundred and twenty-two.

HUGH W. SANFORD.